

Patented Sept. 25, 1923.

1,468,959

# UNITED STATES PATENT OFFICE.

ALBERT L. CLAPP, OF DANVERS, MASSACHUSETTS.

## WATERPROOF PAPER BOARD.

No Drawing.

Application filed June 12, 1922. Serial No. 567,752.

To all whom it may concern:

Be it known that I, ALBERT L. CLAPP, a citizen of the United States, residing at Danvers, in the county of Essex and State 5 of Massachusetts, have invented new and useful Improvements in Waterproof Paper Board, of which the following is a specification.

The object of this invention is to provide 10 a paper board or box board which is highly waterproof and which has a smooth glassy exterior finish at least on one face and is adapted for use in the manufacture of cartons or boxes so that the contents thereof 15 may be maintained in the same condition in which they were introduced into the container or box and without material gain or loss in moisture.

A further object of the invention is to 20 provide a process by which the paper or board may be produced on a paper machine continuously.

In carrying out my invention, while it is 25 possible to form the board of a single layer of waterproof material, I preferably form 30 it in a plurality of layers, the outer or bottom layer of which is formed of the waterproof material.

As the waterproofing agent, I employ 35 Montan wax, crushed or powdered into a finely divided state, which is mixed with the paper stock in the beating engine. This alone cannot be precipitated by the use of usual precipitating agents, such as alum, so 40 that, in order to produce a more or less flocculent precipitate when a suitable agent is employed, I add to the fibrous stock during the beating operation a certain amount of fine hydrated lime,  $-\text{Ca}(\text{OH})_2$ . Apparently a slight chemical reaction results when the lime is brought into contact with the Montan wax, leaving a large proportion of the Montan wax in a free state, but this chemical reaction is sufficient to cause the 45 Montan wax and the precipitate to be thrown down together on the fiber when a precipitant is added. I have found that by the addition of lime there is a coagulating action and a desirable flocculence of the 50 precipitate is secured after the precipitating agent is added to the "furnish." In producing a waterproof material, any suitable fibrous material is placed in the beater with sufficient warm water to ensure its circulation. I may, for example, utilize chemical 55 or ground wood pulp, mixed papers or other

fibrous material used in paper making. Thus I may place in the beater 100 parts by weight of mixed papers and water, heated to a temperature of approximately 110° 60 to 120° F., in sufficient quantity to ensure the circulation of the stock, and at the same time I add 2 parts by weight of finely divided calcium hydroxide. By using warm water the chemical reaction of the 65 lime and the Montan wax is increased, thereby increasing the volume of the precipitate. With the roll adjusted down to the bed plate, the contents of the beater are subjected to hard beating for about 15 minutes until the paper is disintegrated and the 70 fibers separated, and the lime in suspension is thoroughly mixed with the fibrous mass. I then add approximately 20 parts by weight of powdered Montan wax. Preferably 75 this ingredient is in the state of fine subdivision so that it will pass through a sieve of about 40 to 60 mesh. With the roll still adjusted down to the bed plate, the contents of the beater are beaten hard for about 80 30 minutes, the water being maintained at about the same temperature as before. This beating operation effectively distributes the Montan wax throughout the pulpy 85 mass and continues the further disintegration of the fibers. I now add sufficient alum to effect the precipitation of the lime and Montan wax, and, adjusting the roll from the bed plate so that it will not cut the fiber but brush the same, I continue the beater in 90 operation for approximately 30 minutes. A pulp or stock is now produced in which the Montan wax is precipitated on or fixed to the fibers to a greater or less extent and may be formed into a web without loss of 95 the Montan wax.

While the "furnish" thus described is 100 eminently satisfactory for many purposes, I find that still better results may be secured by adding to the beater stock, previous to the addition of the precipitating agent, rosin size or silicate of soda or both. For example, after the Montan wax has been added to the beater contents and the stock is beaten for 30 minutes, I may add 5 parts 105 by weight of sodium silicate and 5 parts by weight of sodium resinate, after which the stock is beaten for 15 minutes. Thereafter I add 10 parts by weight of alum, and, adjusting the roll so that it will brush the 110 fibers, continue the operation of the beater for approximately 30 minutes. By the ad-

dition of silicate of soda or rosin size or both, the volume and the flocculency of the precipitate are increased and the Montan wax is caused to adhere to the fibers. From 5 this stock, a sheet is formed by means of any suitable paper-making machine, such as a cylinder machine, and is dried on the usual drier rolls. Preferably these rolls are heated to a temperature at which the particles of Montan wax are softened or melted 10 so as to permeate any open interstices in the sheet and to fuse together or coalesce. After being dried, the sheet is preferably calendered by calender rolls, as a result of 15 which it presents a smooth glassy exterior surface. The sheet practically does not absorb water to any appreciable extent and is substantially water and moisture proof. The Montan wax is present in such small 20 proportions that the sheet may be bent or creased without readily cracking or breaking.

While a sheet formed of a single layer of 25 waterproof material as thus described may be utilized for many purposes, I preferably form a composite sheet of two or more adherent plies by the use of a multi-cylinder machine. In making a two-ply or a three-ply board, for example, the additional layers 30 or laminations may be formed of any suitable fibrous stock. In producing a three-ply board which may be bent or creased without breaking and thus be adapted for use in the manufacture of boxes or cartons, the top 35 layer or lamination may be produced from a furnish consisting of approximately 30 parts by weight of bleached sulphite, 40 parts by weight of book cuttings and 30 parts by weight of news print. If this 40 furnish be employed, it, together with sufficient water to ensure its circulation, is beaten for approximately 30 to 45 minutes hard beating. The furnish for the center layer 45 or layers may consist of mixed news paper, in which case it is subjected to hard beating for about 45 minutes more or less.

It is quite evident that any suitable number of cylinders may be utilized for these 50 beater stocks in forming the web. If, for example, a six-cylinder machine is used, the waterproof material may be placed in the vat of one cylinder, the stock of mixed sulphite, book cuttings and news in one cylinder, and the other stock placed in the vats 55 of the remaining cylinders. In such case, assuming that the caliper of the composite sheet is 21—25 points, the bottom layer may be 3—5 points, the top layer 3—5 points and the intermediate layer 15 points. Where a 60 composite sheet is thus formed in a continuous sheet or web, the web is passed through the usual "dry end" of the machine, and then through calender rolls as before described.

While other hard gums or bitumens may 65 be used in lieu of Montan wax, the latter

possesses certain decided advantages. That is to say, it has a relatively low melting point, a short melting-point lag, and when melted has a high degree of penetrability.

In the production of the waterproof material in the beater, I regard it as exceedingly desirable that the beating should be continued for a substantial time after the precipitating agent has been added to the stock. I have found that the best results are secured 70 by continuing the beating or "brushing" for at least 25 to 30 minutes.

It has heretofore been proposed to add gilsonite or other hard friable asphalts or bitumens to paper stock in the formation of 80 a sheet, but the sheets thus produced are decidedly unlike one produced as herein described. By the addition of the calcium hydroxide to the Montan wax and the employment of a precipitating agent either with or 85 without sodium silicate, rosin size or the like, I am able to secure a more even distribution of the Montan wax through the pulpy mass and its attachment to the individual fibers due to the voluminous and flocculent precipitate formed. It is important that the precipitate as it is thrown down should be in a 90 flocculent coagulated condition, and, as previously stated, this is increased by the use of lime or its equivalent, and metallic- 95 salt precipitating agent.

By the production of a composite sheet having the water-proof and moisture-proof bottom layer, it is possible to manufacture 100 the cartons with this layer or lining, as it were, on the inner surface of the box walls so that the outer walls may receive the printing or advertising matter which is usually placed on such cartons.

By the formation of a waterproof ply or 105 layer, as herein first described, the composite sheet is flat and does not curl or blister. This is due to the flocculent precipitate and to the increased or prolonged beating after the precipitating agent has been added.

One of the advantages of the improvements herein described is that the waterproof layer of the composite sheet is so 110 highly waterproof that it can be formed in a very thin layer,—even .002 to .003 inch,— 115 and thus enable one to produce a water-proofed board at very slight expense.

What I claim is:—

1. A process of making waterproof paper or box board, which comprises beating finely 120 divided Montan wax into a pulpy mass of cellulose fiber containing finely divided calcium hydroxide, adding a precipitating agent, and forming the pulpy mass into a sheet or web.

2. A process of making waterproof paper or box board, which comprises beating a mass of cellulose fiber and finely divided lime in 125 warm water, adding finely divided Montan wax to and distributing the same throughout 130

the mass, adding a precipitating agent, and then forming the pulpy mass into a sheet or web.

3. A process of making waterproof paper or box board, comprising beating cellulose fiber (100 parts) and lime (2 parts) in warm water; adding Montan wax (20 parts) to and distributing it throughout the pulpy mass; adding alum to cause the precipitation of a flocculent precipitate, and forming the mass into a web or sheet.

4. A process of making waterproof paper or box board, comprising beating cellulose fiber (100 parts) and lime (2 parts) in warm water; adding Montan wax (20 parts) to and distributing it throughout the pulpy mass; mixing rosin size and silicate of soda (5 parts of each) with said mass; adding a precipitating agent to and distributing the same throughout the mass, and then forming the pulp into a web or sheet.

5. A process of making waterproof paper or box board, which comprises beating finely divided Montan wax into a pulpy mass of cellulose fiber containing finely divided calcium hydroxide, adding a precipitating agent, forming the pulpy mass into a sheet or web, and drying said sheet at a temperature sufficient to flux the contained Montan wax.

30 6. A process of making waterproof paper or box board, which comprises beating finely divided Montan wax into a pulpy mass of cellulose fiber containing finely divided calcium hydroxide, adding a precipitating agent, forming the pulpy mass into a sheet or web, drying said sheet at a temperature sufficient to flux the contained Montan wax, and finely calendering the sheet to glaze the surface thereof.

40 7. A process of making waterproof paper or box board, which comprises beating a mass of cellulose fiber and finely divided lime in warm water, adding finely divided Montan wax to and distributing the same throughout

the mass, adding a precipitating agent, then forming the pulpy mass into a sheet or web, and drying said sheet at a temperature sufficient to flux the contained Montan wax.

8. A process of making waterproof paper or box board, comprising beating cellulose fiber (100 parts) and lime (2 parts) in warm water; adding Montan wax (20 parts) to and distributing it throughout the pulpy mass; adding alum to cause the precipitation of a flocculent precipitate, forming the mass into a web or sheet; progressively drying said sheet at a temperature sufficient to flux the contained Montan wax, and finally calendering the sheet to glaze the surface thereof.

9. A process of forming a composite sheet having an exterior waterproof ply or layer, which comprises beating Montan wax into a mass of cellulose fibers and lime, and adding alum to thereby precipitate a coagulant and flocculent precipitate on the fibers; pulping a second mass of paper stock, then bringing webs of such masses into adherent facial contact, and felting and drying the sheet thus formed.

10. A glazed-surface waterproof paper or box board comprising felted cellulose fiber, Montan wax and an insoluble flocculent precipitate.

11. A composite paper or box board, comprising a layer of felted fiber, and an adherent exterior thin highly-waterproof layer of fiber, Montan wax and a voluminous flocculent precipitate.

12. A composite paper or box board, comprising a layer of felted fiber, and an adherent exterior thin highly-waterproof layer of fiber, Montan wax and a voluminous flocculent precipitate, said layer not exceeding two to three one-thousandths of an inch in thickness.

In testimony whereof I have affixed my signature.

ALBERT L. CLAPP.